

## UNITED STATES PATENT OFFICE

2,620,068

DEPRESSION OF COPPER MINERALS FROM  
ORES AND CONCENTRATES

Charles Francis Allen and Robert Ben Booth,  
Stamford, Conn., assignors to American Cyanamid Company, New York, N. Y., a corporation  
of Maine

No Drawing. Application August 16, 1951,  
Serial No. 242,184

15 Claims. (Cl. 209—167)

1

This invention relates to an improved process of froth flotation of sulfide ores and more particularly for the depression of copper minerals in such processes.

Differential flotation processes for the beneficiation of sulfide minerals have been used extensively. The most common processes involve the treatment of lead-zinc ores and lead-copper-zinc ores and depend on the depression of zinc and iron sulfides by ordinary cyanides of the alkali and alkaline earth metals. Zinc sulfate has also been used. When lead and copper sulfides or copper and molybdenum sulfides occur together they are ordinarily obtained as a concentrate by a bulk copper-lead or copper-molybdenum float. The separation of copper sulfides from lead sulfides or from molybdenum sulfides presents a serious problem, particularly the former. Molybdenum sulfides have been floated away from copper sulfides in the past by using molybdenite collectors such as hydrocarbons which are not good collectors for copper sulfide. This has proved an acceptable, though not ideal, solution with certain of these mixed ores. Certain inorganic phosphate compounds have also been used effectively as depressants in the separation of copper sulfides from molybdenum sulfides.

Attempts have been made to depress copper minerals in lead-copper and copper-molybdenum concentrates by the use of cyanides. However, ordinary cyanides, which are effective as depressants for zinc sulfides, have either no selective action in the case of lead-copper concentrates or are too weakly selective to be of practical utility.

According to the present invention, we have found with a certain combination involving certain metals, the cyanide radical and ammonia in a particular state of combination have great selective depressant power for copper minerals, without seriously depressing either lead or molybdenum sulfides. The combination requires the cyanide radical, a metal selected from the group consisting of magnesium, zinc and aluminum, and ammonia in the form of a free base. When these three conditions are satisfied, good selective depressant action for copper sulfides is achieved.

It is not known why the particular chemical constituents must all be present and especially it is not known why the ammonium radical is not useful if it is present as a salt with ordinary stable chemical ionic valence linkages. Thus, for example, ammonium zinc cyanide, which is a definite chemical compound, has substantially no depressant action, although the three required constituents are present in a single compound.

2

The salt-like chemical union of the ammonia with the cyanide defeats any depressing action. As the exact reason for the peculiar requirements for the depressant of the present invention is not known, no theory is advanced as to why the depressants of the present invention act as they do, and the invention is not intended to be restricted to any theoretical explanations.

10 A wide number of compounds or mixtures may be usable for the present invention. For example, the metal may be present as a salt, the cyanide as an alkaline metal or alkaline earth metal cyanide, and the ammonia as ammonium hydroxide or compounds liberating it in flotation operation. This mixture, which may perhaps react in the flotation pulp, gives satisfactory depression. It is also possible to associate the ammonia with either the metal compound or with the cyanide. Thus, for example, a salt of zinc, magnesium or aluminum may be treated with gaseous ammonia with resultant absorption of ammonia in a form which is apparently not normally ionically bound as a complex salt, and this ammoniated salt may then be mixed with any of the commercially available cyanides. A third method involves ammoniating the cyanide and mixing it with a salt of zinc, magnesium, or aluminum. The fourth method, which produces the cheapest and most active depressant, involves the ammoniating of zinc cyanide. This fourth process is not applicable to depressants in which the metal is aluminum because of the notable instability of aluminum cyanide.

35 The proportions of the ingredients are not critical. It is desirable to operate with equimolar amounts of the metal and cyanide. The amount of ammonia in the basic form may vary widely and usually is determined by the amount of ammonia which either the metal salt or the cyanide will take up.

40 The total amount of depressants will vary and is usually figured on the metal cyanide mole equivalent from 2 to 5 lbs./ton of flotation feed in the case of lead-copper concentrates. Some-  
45 what more up to as much as 15 lbs./ton of depressant may be used in the case of copper-molybdenum concentrates. The ranges are practical ranges, there being no sharp cut-off. Amounts below 2 lbs./ton of feed show a falling-off in depressant action which soon makes the operation uneconomical. On the other hand, particularly in the case of lead-copper concentrates, depression of lead sulfides occurs when the amount of depressant is excessive. In most cases  
50 there is no serious loss of lead up to 5 lbs./ton

of feed but the upper limit will vary somewhat with different ores and different concentrates.

The invention has been described in connection with concentrates containing lead and copper sulfides or lead and molybdenum sulfides. It is not limited to concentrates from ores which contain no other metals. Thus, for example, when a lead-copper concentrate is obtained by the froth flotation of lead-copper-zinc ores using the conventional ordinary cyanides as zinc depressants, such a concentrate can be treated by the present invention with the same effectiveness. In general, the process of the present invention is of particular interest in the treatment of concentrates. It is, however, not limited thereto, and in certain cases may be used with the original ore. Ordinarily this is less desirable as the reagent consumption based on the amount of copper and lead present is higher than when concentrates are treated, particularly if the ore is not very high grade.

It is an advantage of the present invention that the flotation operation itself is not changed by the use of the depressants of the present invention. Thus, the ordinary collectors for copper and lead sulfides such as xanthates, dithiophosphates and the like may be used with conventional frothing agents. Ordinary froth flotation operating techniques are also followed, a number of flotation machines in a string, period of flotation in each machine, cleaning and re-cleaning of concentrates where necessary, all following conventional lines and no new operating techniques need to be learned in order to obtain the advantages of the differential flotation which forms the subject matter of the present invention.

As has been pointed out above, some of the depressants of the present invention are physical mixtures and others single constituents. In the case of some of the latter the depressants are themselves new compounds and in a more specific aspect of the present invention are included.

The invention will be described in greater detail in conjunction with the following specific examples, which illustrate typical modifications of the present invention used with representative ores.

All flotation tests were effected in laboratory Fagergren flotation machines under normal flotation conditions:

#### Example 1

Concentrates from a South African lead-copper ore were prepared, having an average assay of about 56.5% lead and 12% copper, the ratio of concentration being approximately three to one. The concentrate was prepared using 0.1 lb./ton of sodium isopropyl xanthate and 0.07 lb./ton of a higher alcohol frother averaging 7 carbons in chain length. The reagents adhering to the concentrate were sufficient to act as a collector-frother for the lead in the succeeding operation. No additional reagents were required.

The concentrate was conditioned with 6 lbs./ton of ammoniated zinc cyanide which was prepared by ammoniating zinc cyanide with gaseous NH<sub>3</sub>, producing a product having the composition Zn(CN)<sub>2</sub>·1.8NH<sub>3</sub>. The concentrate was conditioned and floated in a flotation machine with 0.06 lb./ton of paraffin alcohol averaging seven carbon atoms as a frother to produce a rougher lead concentrate. The concentrate was then conditioned with 0.6 lb./ton of zinc cyanide am-

moniate and 0.06 lb./ton of frother floated to produce a cleaner concentrate.

The ammoniated zinc cyanide may vary in its ammoniated content over a wide range without materially affecting flotation results.

#### Example 2

The concentrate of Example 1 was conditioned with 13.8 lbs./ton of zinc cyanide and 7.5 lbs./ton of ammonium hydroxide containing 25% NH<sub>3</sub>, 0.06 lb./ton of the frother of Example 1 was added and a rougher concentrate obtained.

#### Example 3

The concentrate of Example 1 was conditioned with 21.8 lbs./ton of crude calcium cyanide sold by the American Cyanamid Company as "Aero Brand" cyanide, 25 lbs./ton of ZnSO<sub>4</sub>·H<sub>2</sub>O and 9 lbs./ton of ammonium phosphate. 0.03 lb./ton of frother was then added and a lead concentrate obtained by froth flotation.

The cyanide used contains a large excess of lime which reacts with the ammonium phosphate to liberate ammonia.

#### Example 4

The concentrate of Example 1 was conditioned with 21.5 lbs./ton of "Aero Brand" cyanide, 5.55 lbs./ton of zinc oxide and 22.5 lbs./ton of ammonium phosphate. 0.03 lb./ton of frother was added and a lead concentrate floated. The mixture of "Aero Brand" cyanide and zinc oxide produces zinc cyanide in solution and is sold to the mining trade as a mixture.

When the above procedure was repeated, neutralizing excess lime with ammonium sulfate so that no ammonia is liberated from the ammonium phosphate no useful depression of copper sulfide resulted.

#### Example 5

A concentrate of Example 1 is conditioned with 19 lbs./ton of zinc sulfate, 12 lbs./ton of sodium cyanide and 7.5 lbs./ton of 25% ammonium hydroxide. 0.06 lb./ton of frother was added, and a lead concentrate obtained by froth flotation.

#### Example 6

The concentrate of Example 1 was conditioned with 5.1 lbs./ton of "Aero Brand" cyanide and 4.5 lbs./ton of zinc chloride ammoniated to take up 4 moles of ammonia. 0.06 lb./ton of frother was then added and a lead concentrate floated.

#### Example 7

The concentrate of Example 1 was conditioned with 5.1 lbs./ton of "Aero Brand" cyanide, and 7.2 lbs./ton of zinc sulfate ammoniated to take up 4 moles of ammonia. 0.06 lb./ton of frother was then added and a rougher lead concentrate floated. This was then cleaned after the additional 0.06 lb./ton of frother, and a cleaner concentrate obtained.

#### Example 8

The concentrate of Example 1 was conditioned with 3.1 lbs./ton of "Aero Brand" cyanide, 4.2 lbs./ton of MgCl<sub>2</sub>·6H<sub>2</sub>O ammoniated to add 25% ammonia by weight. 0.06 lb./ton of frother was then added and a lead concentrate floated.

#### Example 9

The concentrate of Example 1 was conditioned with 3.1 lbs./ton of "Aero Brand" cyanide and 5.3 lbs./ton of MgSO<sub>4</sub>·7H<sub>2</sub>O ammoniated to take up

37 parts by weight of ammonia, 0.06 lb./ton of frother was then added and a lead concentrate floated.

*Example 10*

The concentrate of Example 1 was conditioned with 5.1 lbs./ton of ammoniated "Aero Brand" cyanide, the cyanide taking up 11.5% of NH<sub>3</sub> and 11.1 lbs./ton of ammoniated aluminum sulfate containing 18 moles of water, the ammonia absorption amounting to 1/6 by weight. 0.06 lb./ton of frother was then added and the lead concentrate floated.

*Example 11*

The concentrate of Example 1 was conditioned with 11.6 lbs./ton of ammoniated "Aero Brand" cyanide prepared as described in the preceding example and 10.8 lbs./ton of ZnSO<sub>4</sub>·7H<sub>2</sub>O. 0.06 lb./ton of frother was then added and a lead concentrate then floated.

*Example 12*

The concentrate of Example 1 was conditioned with 5.8 lbs./ton of ammoniated "Aero Brand" cyanide prepared as described in Example 10 and 7.3 lbs./ton of ammoniated zinc sulfate prepared as described in Example 7. 0.03 lb./ton of frother was added and a lead concentrate floated.

Metallurgical results of Examples 1 to 12 are shown in the following table which also includes controls where cyanide zinc oxide were used and where cyanide and ammonium hydroxide were used. In the column under depressant, "Aero Brand" cyanide is abbreviated "ABC," zinc magnesium and aluminum salts are written without water of crystallization. Ammoniation is indicated by NH<sub>3</sub>. The assays are given for the final lead concentrate. This is the rougher concentrate in some examples, and the cleaner concentrate where cleaning is described.

| Example | Depressant                                                                            | Assay |     | Percent Dis-<br>tribution |      |
|---------|---------------------------------------------------------------------------------------|-------|-----|---------------------------|------|
|         |                                                                                       | Pb    | Cu  | Pb                        | Cu   |
| 1.      | Zn(CN) <sub>2</sub> ;NH <sub>3</sub>                                                  | 72.3  | 3.4 | 82.1                      | 18.4 |
| 2.      | Zn(CN) <sub>2</sub> ;NH <sub>4</sub> OH                                               | 69.7  | 4.8 | 96.2                      | 32.4 |
| 3.      | ABC;ZnSO <sub>4</sub> ;Ammonium Phosphate                                             | 65.1  | 5.6 | 95.6                      | 39.4 |
| 4.      | ABC;ZnO;Ammonium Phosphate                                                            | 68.4  | 3.2 | 88.4                      | 18.5 |
| 5.      | ZnSO <sub>4</sub> ;NaCN;NH <sub>4</sub> OH                                            | 67.4  | 6.0 | 95.3                      | 37.8 |
| 6.      | ABC;ZnCl <sub>2</sub> ;NH <sub>3</sub>                                                | 65.2  | 6.6 | 95.5                      | 47.2 |
| 7.      | ABC;ZnSO <sub>4</sub> ;NH <sub>3</sub>                                                | 71.7  | 4.0 | 81.8                      | 21.3 |
| 8.      | ABC;MgCl <sub>2</sub> ;NH <sub>3</sub>                                                | 65.9  | 6.0 | 92.7                      | 40.9 |
| 9.      | ABC;MgSO <sub>4</sub> ;NH <sub>3</sub>                                                | 66.1  | 7.7 | 90.7                      | 51.5 |
| 10.     | ABC;NH <sub>3</sub> ;Al <sub>2</sub> (SO <sub>4</sub> ) <sub>3</sub> ;NH <sub>3</sub> | 70.7  | 3.6 | 90.3                      | 22.5 |
| 11.     | ABC;NH <sub>3</sub> ;ZnSO <sub>4</sub>                                                | 65.7  | 5.6 | 96.1                      | 40.5 |
| 12.     | ABC;NH <sub>3</sub> ;ZnSO <sub>4</sub> ;NH <sub>3</sub>                               | 66.4  | 6.9 | 91.1                      | 44.9 |
| Control | ABC;ZnO                                                                               | 47.9  | 7.6 | 4.8                       | 4.53 |
| Control | NaCN;NH <sub>4</sub> OH                                                               | (1)   | (1) | (1)                       | (1)  |

<sup>1</sup> All minerals substantially completely depressed.

*Example 13*

A copper-lead ore from a Chilean mine was ground and conditioned with 0.17 lb./ton of a collector which was a mixture of sodium mercaptobenzothiazole and sodium dissecondary butyl dithiophosphate and 0.06 lb./ton of the 7-carbon atom alcohol frother used in previous examples. The conditioned pulp was floated to give a lead-copper concentrate assaying 9.5% Pb and 17.8% Cu; the ratio of concentration was 14 into 1. This concentrate was then conditioned with 8.0 lbs./ton ammoniated zinc cyanide prepared as described in Example 1 and floated to produce a lead concentrate. 0.06 lb./ton of the alcohol frother used in Examples 1-12 was used;

no additional collector was required. The resulting lead concentrate was cleaned to give a final concentrate assaying 26.7% Pb and 17.9% Cu with a lead recovery of 80.7%.

*Example 14*

A copper molybdenum concentrate from a southwestern ore having an average assay of about 1.85% molybdenite and 30% copper was conditioned with 4 lbs./ton of ammoniated zinc cyanide prepared as described in Example 1; and 0.04 lb./ton of a higher alcohol frother stabilized with fuel oil, which also acts as a molybdenite collector as well as a frother. A molybdenum concentrate was floated which was cleaned and recleaned. An additional 2.0 lbs./ton of ammoniated zinc cyanide was added during the first float and first cleaner float and 1.0 lb./ton during the recleaner float. Each float had the same amount of frother added, 0.04 lb./ton.

A molybdenite concentrate was obtained assay-ing 20.55% MoS<sub>2</sub> Cu. The percentage distribution of MoS<sub>2</sub> was 75.23 in the molybdenite concentrate.

When the concentrate of Example 14 was conditioned with 10 lbs./ton of "Aero Brand" cyanide or 10 lbs. of "Aero Brand" cyanide and 10 lbs. of NH<sub>4</sub>OH no practical copper depression resulted.

*Example 15*

A copper molybdenite concentrate from a Utah copper ore having an average assay of 1.68% MoS<sub>2</sub> and 30% copper, prepared by froth flotation using dicrosetyl dithiophosphate as a collector, was conditioned with 5 lbs./ton of ammoniated zinc cyanide, prepared as described in Example 1, and then floated with 0.06 lb. of the frother of Example 13. The concentrate was cleaned 6 times, additional ammoniated zinc cyanide for the first float and six cleanings in pounds per

ton being as follows: 2.5, 3.0, 2.0, 1.0, 1.5 and none.

Each flotation operation involved the addition of the same amount of frother, 0.06 lb./ton. The distribution of molybdenite in the 6th cleaner

concentrate was 83.1% and this concentrate con-tained 36.6% MoS<sub>2</sub> and only 3.64% Cu, the re-mainder of the concentrate being a fine sericitic material. The copper product (the final tailing) contained only 0.05% MoS<sub>2</sub>.

We claim:

1. A process of selectively depressing copper sulfides in the presence of a sulfide included in the group consisting of lead sulfides and molybdenum sulfides which comprises effecting froth flotation in the presence of a collector for sul-

fides and from 2 to 15 lbs./ton of a depressant containing the cyanide radical, a cation selected from the group consisting of zinc magnesium and aluminum, and non-ionically linked ammonia.

2. A process according to claim 1 in which the copper sulfides are associated with lead sulfides.

3. A process according to claim 2 in which the depressant comprises ammoniated zinc cyanide.

4. A process according to claim 1 in which the sulfide associated with the copper sulfides is molybdenite.

5. A process according to claim 4 in which the depressant comprises ammoniated zinc cyanide.

6. A process according to claim 1 in which the depressant is a mixture of an ammoniated salt containing the cation and a soluble cyanide.

7. A process according to claim 6 in which the soluble cyanide is a crude calcium cyanide containing excess lime.

8. A process according to claim 7 in which the sulfides associated with the copper sulfides are lead sulfides.

9. A process according to claim 6 in which the sulfides associated with the copper sulfides are lead sulfides.

10. A process according to claim 1 in which the cation is zinc.

11. A process according to claim 10 in which the sulfides associated with the copper sulfides are lead sulfides.

12. A process according to claim 1 in which the cation is magnesium.

13. A process according to claim 12 in which the sulfides associated with the copper sulfides are lead sulfides.

14. A process according to claim 1 in which the cation is aluminum.

15. A process according to claim 14 in which the sulfides associated with the copper sulfides are lead sulfides.

CHARLES FRANCIS ALLEN.  
ROBERT BEN BOOTH.

#### REFERENCES CITED

The following references are of record in the file of this patent:

#### UNITED STATES PATENTS

|    | Number    | Name          | Date           |
|----|-----------|---------------|----------------|
| 15 | 1,429,544 | Stevens       | Sept. 19, 1922 |
|    | 1,552,936 | McArthur, Jr. | Sept. 8, 1925  |
|    | 1,596,120 | Poindexter    | Aug. 17, 1926  |
|    | 1,609,038 | Olberg        | Nov. 30, 1926  |
|    | 1,735,190 | Warren        | Nov. 12, 1929  |
|    | 1,939,068 | Lemmon        | Dec. 12, 1933  |
|    | 1,974,218 | Ruth, Jr.     | Sept. 18, 1934 |
|    | 2,105,901 | Brinker       | Jan. 18, 1938  |

#### FOREIGN PATENTS

|    | Number  | Country       | Date         |
|----|---------|---------------|--------------|
| 25 | 607,731 | Great Britain | Oct. 6, 1948 |

#### OTHER REFERENCES

30 Hoffman, "Lexikon der Anorganischen Verbindungen," Band 1 (Nos. 1-31), pages 554, 558. Published by Verlag Von Johann Ambrosius Barth, Leipzig, Germany, 1917.